



US006877206B2

(12) **United States Patent**  
Hall et al.

(10) Patent No.: **US 6,877,206 B2**  
(45) Date of Patent: **Apr. 12, 2005**

(54) **METHOD FOR PRODUCING A METAL STRIP**

(75) Inventors: **Dan Hall**, Powell, OH (US); **Iippo Koppinen**, Pori (FI); **George Mayer**, Delaware, OH (US); **Brian Swank**, Marengo, OH (US)

(73) Assignee: **Outokumpu Oyj**, Espoo (FI)

(\*) Notice: Subject to any disclaimer, the term of this patent is extended or adjusted under 35 U.S.C. 154(b) by 142 days.

(21) Appl. No.: **10/199,768**

(22) Filed: **Jul. 19, 2002**

(65) **Prior Publication Data**

US 2004/0011109 A1 Jan. 22, 2004

(51) Int. Cl.<sup>7</sup> ..... **B21B 1/46**

(52) U.S. Cl. ..... **29/527.7; 72/252.5**

(58) Field of Search ..... 29/527.7; 72/234, 72/366.2, 377, 204, 252.5

(56) **References Cited**

## U.S. PATENT DOCUMENTS

2,371,671 A \* 3/1945 Blount, et al. ..... 72/366.2

4,232,727 A \* 11/1980 Bower et al. ..... 164/76.1  
4,233,832 A 11/1980 Rowell  
4,519,118 A \* 5/1985 Shinopoulos et al. ..... 492/1  
4,793,169 A 12/1988 Ginzburg  
5,119,660 A 6/1992 Koppinen et al.  
6,813,921 B2 \* 11/2004 Hall et al. ..... 72/234

\* cited by examiner

Primary Examiner—Lowell A. Larson

(74) Attorney, Agent, or Firm—Morgan & Finnegan, LLP

(57) **ABSTRACT**

The invention relates to a method for producing a metal strip from a cast by rolling in which method the technique of a profiled rolling in combination with a strip rolling is used. The material for the metal strip is first cast by using a casting technique to produce a cast profile having the center part thicker than the lateral parts and the cast profile is in an essentially continuous manner conducted into a rolling mill where during the at least two-staged profiled rolling the cast profile is divided into two symmetrical segments and maintained as two equal segments. These segments are spread into the lateral regions of the material to be rolled into a flattened profile which is as an object for at least one-staged strip rolling so that the spread ratios between the center part dimension of the cast profile and the width of the strip of greater than 2.8:1 are achieved.

**12 Claims, 4 Drawing Sheets**







Fig. 2      Fig. 3

Fig. 4

Fig. 5



Fig. 6



Fig. 7

Fig. 8

Fig. 9

Fig. 10

## METHOD FOR PRODUCING A METAL STRIP

This relates to a method for producing a metal strip from a casting by rolling and annealing.

The U.S. Pat. No. 5,119,660 relates to a method for manufacturing metal objects, particularly non-ferrous metal objects, by means of extrusion. In this method the material is fed as cast from the caster to an extrusion device. The casting is a rod, which is cast by upwards casting in a separate location and has a coarse-grained cast structure. The casting is fed to the extrusion device, which is preferably a continuous extrusion device where the rod is fed into a groove of a rotating Conform extrusion wheel. The frictional grip pushes the rod against a fixed abutment and the shear action on the material generates a sufficient pressure and temperature to extrude the material through a die to form a shaped product. The shaped product can preferably be a continuous length strip, which is wound on large coils. The product has proven to be a major cost-savings and allowing eliminate cross-welding of traditional pancake coils, improving weld quality and increasing line speeds. Nevertheless, the continuous extrusion used in the method of U.S. Pat. No. 5,119,660 for a continuous strip is not so reliable as expected. Further, the strip produced by the continuous extrusion has a small spread ratio, i.e. the ratio between the final width of the strip and the original diameter of the cast from the caster.

In the case of rolling a metal rod into a metal strip, the final strip width is dependent upon the work roll diameter, lubrication, and the diameter of the rod. The current limiting factors for processing a metal rod into a metal strip are the small spread ratios (width/diameter) and controlling the edge variation. With small spread ratios the ability to produce a wide metal strip from a metal rod becomes marginally feasible due to the size of the equipment needed. Also as the diameter of the rod increases so does the amount of the edge variation encountered in the process. When considering a process for manufacturing a metal strip from a metal rod, the easiest approach is to do a direct reduction of the rod and obtain a given width. Normally the width of the metal strip (i.e. copper) processed by the direct reduction method has a spread ratio of 1.7:1-1.9:1. By simply striking a line across the diameter of a rod and multiplying it by 1.7 a final strip width can be determined. In order to achieve higher spread ratios from a given diameter of rod, it is necessary to find a method that will extend the initial line length through the rod. The theoretical maximum width that can be achieved from a rod is obtained by striking a helical arc through the material. If the rod were to be uncoiled about the arc the theoretical maximum width of strip could be achieved for a given thickness. Although this would produce the maximum width of strip there are fundamental problems preventing this process from being exploited.

From the U.S. Pat. No. 4,793,169 it is known a continuous rolling mill in which a thin slab from a continuous caster can be processed to a strip through the hot rolling mill without interruption. In one embodiment of this U.S. Pat. No. 4,793,169 billets or shapes having curved cross sections such as rounds and ovals may be rolled. The work rolls have complementary, diverging work surfaces, each beginning with a narrow region at the midpoint of the roll and diverging to a wider region extending across the width of the roll. When the wider regions come into contact with the material, the roll gap is relieved and the rolled material is partially retracted in a back pass. The roll gap is again closed and the narrow region again contacts the material for further

the flattening and spreading, eventually to produce the strip. While this process can make wide strip its through-put is relatively low and the mechanism to make such a motion complex compared to the conventional rolling mill.

The U.S. Pat. No. 4,233,832 describes a method and apparatus for rolling a metal wire or rod into a wide, flat strip. In this method, the metal wire or rod is passed between two rolls one side the other but with offset axis. The larger outer roll, which may be ring-shaped has a smooth inside contact surface. The smaller internal roll has a smooth outside contact surface. The opposing, smooth surfaces have a separation at the closest point, which is less than  $\frac{1}{3}$  the diameter of the metal wire or rod to be fed between them. The distance between the point, where the wire first contacts the opposing, smooth contact surfaces of the converging throat and the closest point of separation between the opposing surfaces is preferred to be at least four times the original diameter of the wire or rod being fed there through. Rolling of metal wire or rod in this manner produces a wide, flat metal strip having a width of at least 2.5 times the original diameter of the wire or rod, and the resultant strip width may considerably exceed 4.0 times the original diameter. As an example for the U.S. Pat. No. 4,233,832 it is mentioned a wire of nominally pure lead having a diameter of 0.190 of an inch (4.8 mm) was flattened into a strip having a width of approximately 1 inch. This represents a width to diameter ratio of approximately 5.3.

In the referred U.S. Pat. Nos. 4,793,169 and 4,233,832 the rolling for a flattened strip is carried out in a single rolling stage. This requires that the devices and especially the surfaces of the work rolls are well manufactured. Also the maintenance of the devices and the rolls is very difficult in order to keep the tolerance continuously between the rolls essentially the same for instance because of the quality requirements of the strip.

The object of the present invention is to eliminate drawbacks of the prior art and to create an improved method for producing a metal strip starting with a cast wire from a caster and to overcome the current limitation in the spread ratio by a combination of an upwards casting technique with a profiled and strip rolling technique. The essential features of the invention are enlisted in the appended claims.

According to the invention the metal material for a strip is first cast by using a casting technique to produce in an essentially continuous manner a cast, having advantageously a shape of a profile in which the center part of the profile is essentially thicker than the lateral parts of the profile, as a rod or a bar. The casting is advantageously carried out in an essentially horizontal or essentially vertical direction, but the casting can also be carried out in a slant position between the horizontal and vertical position. The cast profile is then in an essentially continuous manner conducted to a rolling mill where the technique of a profiled rolling and strip rolling is used, advantageously directly from the casting device. Thus the cast profile is advantageously as a cast when the first stage of rolling starts. There is then advantageously no working of the cast profile before rolling, and the as-cast material is clearly below any working (i.e. tempering or softening annealing) temperature. However, if needed, at least one working stage is possible to do as continuous operation between the caster and the first rolling stage of the invention.

For the longitudinal and lateral spread of the cast profile for a metal strip in accordance with the invention the cast profile is advantageously divided by rolling into two symmetrical segments and maintained as two equal segments until the cast profile is rolled to a flattened strip.

In one preferred embodiment of the invention during the initial rolling operation the cast profile is split into two symmetrical segments using an approach that is similar to driving a wedge into a piece of wood. The bulk displacement of the cast profile is in the lateral direction due to the relative resistance encountered. The longitudinal elongation with this approach can be maintained below 5%. After the cast profile has been divided into two equal segments, the profiled rolls in the following operations force the bulk movement of the cast profile laterally. With low losses of the cast profile material in the longitudinal direction, spread ratios (width/diameter) between the center part dimension of the cast profile and the width of the strip of greater than 2.8:1 are achieved.

In the method of the invention the cast profile is rolled into a flattened strip by a multistage rolling where at least two stages from the start are based on the profile rolling following by at least one stage of the strip rolling. The rolls for the stages of the profile rolling are shaped so that the rolling effect is focused on the cast profile in its center part so that the center part of the cast profile divides the cast profile to two symmetrical lateral parts having a thickness greater than the center part of the cast profile material.

The cast profile to be rolled is centered so that the cast profile is fed in its center part to the point of the gap between the rolls where the distance between the rolls is the shortest. Thus the rolling advantageously starts from the thickest part of the cast profile. The rolls for the first stage rolling are advantageously so shaped that the surface of the center part of a roll is convex curved. The curved center part of the roll surface is connected at both ends with the surface of the lateral parts of the roll, which are essentially linear and are directed divergently from the center part of the roll. Thus the two rolls are at the closest to each other at the center point of the rolls. The curved part of the roll is between 20 and 35% of the total width of the roll. The surfaces of the lateral parts of the roll form a sharp angle of between 40 and 60 degrees against the rolling plane. Thus the cast profile to be rolled is able to spread towards the lateral regions. The surfaces in the lateral parts of the roll can also be curved if the curves are mainly directed divergently from the center part of the roll.

In the second stage for the profile rolling the roll is shaped so that the convex curved part of the roll in the center part is wider than in the first stage of the profile rolling. Thus the area where the material to be rolled has a mechanical contact with the surfaces of the rolls is also wider and the material is further spread in its lateral regions. The lateral regions of the surface of the roll starting from both ends of the curved center part of the surface of the roll will be linear or curved so that the lateral regions are directed divergently from the center part of the roll.

In another preferred embodiment of the invention the rolls for the first stage rolling are asymmetrical so that the rolling effect is focused to the center part of the cast profile to be rolled. This is carried out so that the surface of the center part of one of the working rolls is convex curved while the other of the working rolls is concave curved. The convex curved center part of the roll surface is between 5 and 20% of the total width of the roll surface. This convex curved center part of the roll surface is connected at both ends with the surface of the lateral parts of the roll, which are concave curved and are directed divergently from the center part of the roll. The concave curved roll is concave curved at least 90% of the total width of roll surface which roll surface is narrower than or equal to the roll surface of the roll having the center part convex curved. Based on the

shapes of the rolls the two rolls are still at the closest to each other at the center point of the rolls. Thus the material to be rolled is able to spread towards the lateral regions.

In the second rolling stage the working roll positioned in a respective manner to the roll having the center part convex curved in the first rolling stage is still convex curved in the center part but the convex center part is larger than in the first rolling stage. The convex curved part is between 20 and 35% of the total width of the roll surface. The convex curved center part of the roll surface is connected at both ends with the surface of the lateral parts of the roll, which are essentially linear and are directed divergently from the center part of the roll. The surfaces of the lateral parts of the roll advantageously form a sharp angle of between 40 and 60 degrees against the rolling plane. The counter working roll for the convex curved roll is in the second stage advantageously essentially flat and the width of the roll surface is essentially equal to the roll surface of the convex curved roll. Thus also in this stage the material to be rolled is able to spread towards the lateral regions.

In the third rolling stage the convex curved working roll is convex curved essentially in the total width of the roll surface. The counter working roll for the convex curved roll is in this stage advantageously essentially flat and the width of the roll surface is advantageously larger than the roll surface of the convex curved roll. The two working rolls are still at the closest to each other at the center point of the rolls and, therefore, the spreading of the material to be rolled towards the lateral regions will continue in this third stage.

Despite of the embodiments described above when the desired width of the strip is achieved the rolling stage or stages will concentrate to the thickness of the rolled strip and thus the rolling surfaces between two working rolls are parallel and the gap between two working rolls is essentially the same for the whole width of the rolling surfaces.

The invention is described in more details referring to following drawings where

FIG. 1 illustrates a schematical side-view of the preferred embodiment of the invention,

FIG. 2 illustrates the embodiment of FIG. 1 from the direction 2—2,

FIG. 3 illustrates the embodiment of FIG. 1 from the direction 3—3,

FIG. 4 illustrates the embodiment of FIG. 1 from the direction 4—4,

FIG. 5 illustrates the embodiment of FIG. 1 from the direction 5—5,

FIG. 6 illustrates a schematical side-view of another preferred embodiment of the invention,

FIG. 7 illustrates the embodiment of FIG. 6 from the direction 7—7,

FIG. 8 illustrates the embodiment of FIG. 6 from the direction 8—8,

FIG. 9 illustrates the embodiment of FIG. 6 from the direction 9—9,

FIG. 10 illustrates the embodiment of FIG. 6 from the direction 10—10.

According to the FIG. 1, the material to be processed for a strip is first melted in the melting furnace 12 and the melt is conducted into a basin 13. The melt material in the basin 13 is cast by drawing the melt in an essentially continuous manner through a die 14 upwards essentially vertically and by simultaneously cooling the melt for a casting 1. The casting 1 profiled in the shape of a rod is further conducted to the first rolling stage 2.

The rod material 1 from the casting to be rolled is fed to the first profile rolling stage 2 where the work rolls 3 are so

shaped that the rolls **3** have the first contact with the rod material **1** in the center part of the rod material **1**. The rolls **3** divide the rod material **1** into two symmetrical segments **4** as shown in FIG. 2. The working rolls **3** are so shaped that the distance between the rolling surfaces of the rolls **3** increases from the center part towards the lateral parts of the rolls **3**. Therefore the segments **4** have space to spread into the lateral directions.

After the first profile rolling **2** the material to be rolled **1** is fed into the second profile rolling stage **5** where the rolling effect is still focused into the center part of the material **1**, but now for a wider region than in the first profile rolling stage **2**. The working rolls **6** in the second profile rolling stage **5** are so shaped that the distance between the rolling surfaces of the rolls **6** is the shortest in the center part and the distance in the center part is essentially similar to the distance between the working rolls **3** in the first profile rolling stage **2**. However, the region in the working rolls **6**, which have mechanical contact with the material **1** to be rolled is wider. Thus the rolls **6** spread the material **1** more and more towards the lateral regions where the segments will be changed so that the width of segments **4** will increase at the expense of the thickness of the material **1** which is still thicker than in the center part.

The material **1** to be rolled is further transferred into the third profile rolling stage **7** where the distance between the working rolls **8** is in the center part of the rolling surface essentially the same as in the preceding rolling stages **2** and **5**. The distance between the working rolls **8** will increase towards the lateral regions of the rolling surfaces, but the contact between the working rolls **8** and the material **2** is at least 80% of the width of the rolling surfaces of the working rolls **8**. Because the material **2** to be rolled has space in the lateral regions to spread, the width of the material **1** will increase accordingly.

After the third profile rolling stage **7** the material **1** to be rolled is flattened so much that the material **1** is ready for a strip rolling stage **9** as shown in FIG. 5. In the strip rolling stage **9** the rolling surfaces of the working rolls **10** are in the essentially same distance from each other at their total width. The mechanical contact between the rolling surfaces of the working rolls **10** and the material **1** is then created for the whole width of the strip **11**. The width of the strip **11** is about 3 times the diameter of the original rod material **1** fed into the method of the invention.

In the other preferred embodiment of the invention illustrated in FIGS. 6-10 the material to be processed for a strip is first melted in the melting furnace **15** and the melt is conducted into a basin **16**. The melt material in the basin **16** is cast by drawing the melt in an essentially continuous manner through a die **17** horizontally and by simultaneously cooling the melt for a casting **26**. The casting **26** profiled in the shape of a rod is further conducted to the first rolling stage **2**.

The the working rolls **21** and **22** in the first profiled rolling stage **23** are so shaped that the rolls **21** and **22** have the first contact with the rod material **26** in the center part of the rod material **26**. The rolls **21** and **22** divide the rod material **26** into two symmetrical segments **32** as shown in FIG. 7. The rolls **21** and **22** for the first rolling stage **23** are so shaped that the surface of the center part of one roll **21** is convex curved while another roll **22** is concave curved. The convex curved center part of the roll surface **24** in the roll **21** is between 5 to 20% of the total width of the roll surface **24**. This convex curved center part of the roll surface **24** is connected at both ends with the surface of the lateral parts of the roll **21**, which are concave curved and are directed

divergently from the center part of the roll. The concave curved roll **22** is concave curved at least 90% of the total width of roll surface **25** which roll surface **25** is narrower than or equal to the roll surface **24** of the roll **21**. Based on the shapes of the rolls **21** and **22** the rolls **21** and **22** are still at the closest to each other at the center point of the roll surfaces **21** and **22**. Thus the segments **32** of the material **26** to be rolled is able to spread towards the lateral regions.

In the second rolling stage **27** the rolling effect is still focused into the center part of the material **26**, but now for a wider region than in the first profile rolling stage **23**. The roll **28** positioned in respective manner to the roll **21** having the center part convex curved in the first rolling stage **23** is still convex curved in the center part but the convex center part is larger than in the first rolling stage **23**. The convex curved center part of the roll **28** is 25% of the total width of the roll surface **29**. The convex curved center part of the roll surface **29** is connected at both ends with the surface of the lateral parts of the roll **28**, which are essentially linear and are directed divergently from the center part of the roll **28**. The surfaces of the lateral parts of the roll **28** advantageously form a sharp angle of at least 45 degrees against the rolling surface. The counter roll **30** for the convex curved roll **28** is in the second stage advantageously essentially flat and the width of the roll surface **31** of the roll **30** is essentially equal to the roll surface **29** of the convex curved roll **28**. Thus also in this stage the material **26** to be rolled is able to spread more and more towards the lateral regions of the roll surfaces **29** and **31**. Then the segments **32** of the material **26** to be rolled will be changed so that the width of segments **32** will increase at the expense of the thickness of the material **26** which is still thicker than in the center part.

In the third rolling stage **33** the working rolls **34** and **35** are so shaped that the rolling effect is still focused into the center part of the material **26** and the material **26** to be rolled has space in the lateral regions to spread. One of the working roll **34** positioned in respective manner as the rolls **21** and **28** in the previous stages to the material **26** to be rolled is convex curved essentially in the total width of the roll surface **36**. The counter roll **35** for the convex curved roll **34** is in this stage advantageously essentially flat and the width of the roll surface **37** is advantageously larger than the roll surface **36** of the convex curved roll **34**. The two working rolls **34** and **35** are still at the closest to each other at the center point of the rolls **34** and **35** and, therefore, the spreading of the material to be rolled towards the lateral regions will continue in this third stage **33**.

After the third profile rolling stage **33** the material **26** to be rolled is flattened so much that the material **26** is ready for a strip rolling stage **38** as shown in FIG. 10. In the strip rolling stage **38** the rolling surfaces **39** and **40** of the working rolls **41** and **42** are in the essentially same distance from each other at their total width. The mechanical contact between the rolling surfaces **39** and **40** of the working rolls **41** and **42** and the material **26** is then created for the whole width of the strip **43**. The width of the strip **43** is about 3 times the diameter of the original rod material **26** fed into the method of the invention.

What is claimed is:

1. Method for producing a metal strip from a cast by rolling, in which method the technique of a profiled rolling in combination with strip wiling is used, the method comprising:

casting material for the metal strip to produce a cast profile having a center part that is thicker than lateral parts thereof;

conveying the cast profile in an essentially continuous manner into a rolling mill, during an at least two-staged profiled rolling;

providing rolling surfaces of the working rolls that include, in cross-section, at least a center portion that is continuously curved;

dividing the cast profile into two symmetrical and equal segments; and

spreading the two equal segments into lateral regions useful for one-staged strip rolling, so that a spread ratio between the width of the strip and a center part dimension of the cast profile is greater than 2.8:1.

2. Method according to claim 1, further comprising casting in an essentially vertical direction.

3. Method according to claim 2, further comprising feeding rod material to be rolled in each rolling stage into a gap between two working rolls.

4. Method according to claim 1, further comprising casting in an essentially horizontal direction.

5. Method according to claim 4, further comprising feeding rod material to be rolled in each rolling stage into a gap between two working rolls.

6. Method according to claim 1, further comprising casting in a slant position.

10

15

20

7. Method according to claim 1, further comprising feeding rod material to be rolled, in each rolling stage, into a gap between two working rolls.

8. Method according to claim 1, further comprising carrying out the rolling stages for the profiled rolling and for the strip rolling in separate rolling devices.

9. Method according to claim 1, further comprising using working rolls in which a rolling surface of a first working roll of each rolling stage is substantially identical to a rolling surface of a second working roll in the same rolling stage.

10. Method according to claim 1, further comprising providing using working rolls in which the shortest distance between rolling surfaces of each pair of working rolls in each profiled rolling stage are substantially equal.

11. Method according to claim 1, further comprising increasing during profiled rolling, stage by stage, a mechanical contact area between the material being rolled and rolling surfaces of the working rolls.

12. Method according to claim 1, further comprising providing rolling surfaces of the working rolls that are, in cross-section at their center parts, convex curved.

\* \* \* \* \*